

## UNITED STATES PATENT OFFICE.

FRANK R. PALMER, OF READING, PENNSYLVANIA, ASSIGNOR TO THE CARPENTER STEEL COMPANY, OF READING, PENNSYLVANIA, A CORPORATION OF NEW JERSEY.

## HIGH-PHOSPHORUS SCALE-RESISTING STEEL.

No Drawing.

Application filed July 10, 1926. Serial No. 121,738.

This invention relates to an improved scale-resisting steel or ferrous alloy intended particularly for the production of shaped articles of manufacture which are required 5 to maintain a stable non-corrosive surface though subjected to high temperatures such as occur in automobile engines and other uses. And it consists essentially in the deliberate provision in the alloy of a content of phosphorus adapted to effectively and economically impart the desired quality thereto without deleterious effect for the intended purposes.

Phosphorus has unintentionally appeared 15 heretofore generally as a recognizedly injurious element; the elimination of it to a maximum content of .05%, being commonly deemed a commercial requirement in alloy steels, as is specifically prescribed for instance in the standard specifications of the Society of Automotive Engineers and the American Society for Testing Materials; though in the simple carbon steels a phosphorus content as high as .125% has been accepted for the securing of greater machine-ability, notwithstanding the generally objectionable brittle quality imparted thereby.

My invention is based upon the discovery and practical development of the fact that 30 phosphorus, heretofore commonly treated as an incidental impurity requiring elimination, may be deliberately employed to determined advantage in percentages which are "high" relative to those ordinarily tolerated in actual manufacture.

The practical development of this discovery, based on extensive experimentation and investigation, has shown that this heretofore commonly worse than worthless element, may be utilized in relatively "high" percentages, even in simple steels, to satisfactorily impart a considerable degree of scale-resistance quality; and that in connection with comparatively small quantities of 45 other elements, as chromium and silicon, heretofore known to impart such quality in alloy steels, it greatly adds to such desired effect, serving not only as an economical and efficient substitute for increased quantity of 50 the relatively expensive element or elements, but carrying such desired effect farther than is attainable by such elements alone.

In more specifically setting forth the invention as developed by considerable experimentation, preliminary statement will be

made in definite percentages, of the content of a ferrous alloy which embodies the invention satisfactorily, and completely as now appears; as follows: carbon .40%; phosphorus .15%; chromium 3.00%; silicon 6.00%; molybdenum .50%.

It is to be understood that the particular formula above specifically noted may be readily varied within the scope of my invention as further described hereinafter and defined in the subjoined claims; that any content of incidental elements, such as manganese and sulphur, is ignored; that the chromium, silicon, and molybdenum contents noted provide a very satisfactory basis for effective use of the high phosphorus content indicated by the preferred percentage noted; that the chromium and silicon contents indicate the preferable restricted use of these known elements when used jointly in connection with my high phosphorus content the chromium content being increased when the silicon is omitted; that the molybdenum element is included as advantageously serving in the present alloy, its known purposes, namely the increasing of the so-called red-hardness and toughness. As to the essential novel element, high phosphorus, the stated content (.15%) is approximating that which has been found to be most efficacious in proportion to the quantity used. It is noted however, that my actual use indicates that any increase in this percentage of phosphorus increases correspondingly though less rapidly the desired scale-resisting quality up to a maximum of approximately .50%—about where also an objectionable brittleness effect is developed; and that decrease of this stated content (.15%) reduces correspondingly though more rapidly the scale-resisting effect produced,—such effect practically disappearing in alloy steels when a less percentage of phosphorus is used than .05%, and being practically unimportant with less than .08%; also that when the high phosphorus content is provided in an otherwise ordinary simple carbon steel, without content of the heretofore known scale-resisting elements as chromium and silicon mentioned, that the percentage of phosphorus provided should be in excess of .125% to provide satisfactory effect and up to .50% as stated.

As indicating the actual scale-resisting effect of deliberately employed phosphorus in relatively high percentages heretofore prac-

tically prohibited, as contemplated by my invention, I mention as examples the following alloy steels among many machined and ground specimens practically tested: the preferred content of carbon, chromium, and silicon stated above being employed in both, with a low phosphorus content in one and a high phosphorus content in the other:

| 10    | Carbon   | Silicon  | Chromium | Phosphorus |
|-------|----------|----------|----------|------------|
|       | Per cent | Per cent | Per cent | Per cent   |
| No. 1 | .40      | 2.00     | 3.00     | 0.047      |
| No. 2 | .40      | 2.00     | 3.00     | .157       |

These specimens being heated to 1600 F., in air, for eight hours, No. 1 acquires a loose peeling scale, while No. 2 shows only a bronze tarnish color with no scale at all. Further tests show that five per cent additional chromium was required to be added to No. 1 in order to make it approach the scale resistance of No. 2; showing great economy in the employment of the high phosphorus content in the latter with equal desired effect.

Having in mind the practical difficulties of accurately determining actual effects of various percentages of the phosphorus, in connection with the use of other elements in various proportions, it will be understood that the main effects are clearly set forth above with full disclosure for practical use; and that the outstanding feature of the invention is the discovery and practical application of the fact that the phosphorus element, which has heretofore been known in steels mainly as an injurious and troublesome impurity and at best as a limitedly tolerable element, may be deliberately employed to produce a much desired product; and this, not only as an inexpensive substitute for much or all of the more expensive elements heretofore used for like purposes, but with higher results than have heretofore been practically attainable at reasonable cost. It will be seen

that while the invention provides for the use of phosphorus only in actually small percentages of the mass, such percentages are so high relative to the percentages heretofore tolerated or permissible in commercial use, as to warrant distinguishing this improved alloy as a "high-phosphorus" steel or ferrous alloy, notwithstanding that such designation runs counter to a strong existing prejudice against such content in commercially desirable steels.

My improved alloy steel can be readily and satisfactorily produced by the usual crucible pot melting method, by compounding with an iron base the ferro alloys ordinarily used for adding the stated elements.

What I claim is:

1. A scale-resisting alloy steel containing carbon less than 1.50%, phosphorus .05 to .50%, chromium 3% to 30%.
2. A scale-resisting alloy steel containing carbon less than 1.50%, phosphorus .05 to .50%, chromium 3% to 30%, molybdenum .10 to 2.00%.
3. A scale-resisting alloy steel containing carbon .05% to 1.50%, phosphorus .05% to .50%, chromium 1.00% to 30.00%, silicon 1.00% to 5.00%.
4. A scale-resisting alloy steel containing carbon .05% to 1.50%, phosphorus .05% to .50%, chromium 1.00% to 30.00%, silicon 1.00% to 5.00% and molybdenum .10% to 2.00%.
5. A scale-resisting alloy steel containing the following elements in approximately the stated proportions, namely, carbon .40%, chromium 3.00%, silicon 2.00%, phosphorus .15%.
6. A scale-resisting alloy steel containing the following elements in approximately the stated proportions, namely, carbon .40%, chromium 3.00%, silicon 2.00%, phosphorus .15%, molybdenum .50%.

In testimony whereof I affix my signature.

FRANK R. PALMER.